

T. B. ROGERSON.  
REGENERATIVE OPEN HEARTH FURNACE.  
APPLICATION FILED FEB. 24, 1914.

1,104,448.

Patented July 21, 1914



*Witnesses:*

W. F. Nagle.  
H. G. Dietrich

Inventor.

By Thomas Bond Rogerson.  
Wiedersheim & Fairbanks  
Attorneys.

# UNITED STATES PATENT OFFICE.

THOMAS BOND ROGERSON, OF TOLLCROSS, GLASGOW, SCOTLAND.

## REGENERATIVE OPEN-HEARTH FURNACE.

1,104,448.

Specification of Letters Patent. Patented July 21, 1914.

Application filed February 24, 1914. Serial No. 820,381.

*To all whom it may concern:*

Be it known that I, THOMAS BOND ROGERSON, a subject of the King of Great Britain, residing at Tollcross, Glasgow, Scotland, 5 have invented certain new and useful Improvements Relating to Regenerative Open-Hearth Furnaces, of which the following is a specification.

This invention relates to regenerative 10 open hearth furnaces.

At present, with such furnaces, when what is technically termed the "block" (i.e. the wall or arch of refractory material having the air and gas ports therein) is 15 burnt, or gives way, it is usual to take the gas off the furnace and allow the furnace to cool down and thereafter re-build the block with bricks. This procedure takes some time, as much as from four days to a week 20 according to the type of furnace, so that, during this period, the furnace is not working, which means a very considerable pecuniary loss. After the furnace has been repaired it is heated up again and can there- 25 after be used as before. The cooling down and reheating of the furnace and checker work is injurious to and tends to shorten the life thereof.

Many devices have been suggested or de- 30 vised with the object of lengthening the useful life of the block but all are costly, many are cumbrous, and others again re- 35 quire constant up-keep. A method adopted is, at considerable expense, to build the block very massively so as to prolong the effective 40 workability of the furnace while, in some instances, for this object, hollow castings, through which water can circulate, are built in the brickwork. In other cases again the whole block is made removable so that, when 45 burnt, or rendered ineffective, it can be lifted out by a crane and then be replaced by another block which is lowered into position. Owing to the trouble and expense con- 50 nected with such methods they have not heretofore been generally adopted. Instead of adopting such methods of overcoming the difficulty I have devised an entirely new method whereby the burned block can be re- 55 paired and lengthened to the desired extent in a very short interval of time, say a few hours, and, what is of very great importance, this repair can be effected without interrupting the operation of the furnace, so 60 of heat during the repair, no loss of output that there is no loss, or practically no loss,

and no cooling and re-heating of the furnace and checker work; further, the repair can be effected without interfering with the working parts of the furnace. The method adopted is simple and its cost is negligible, 60 all the materials used being easily obtained at a low cost, and the repair work can be effected by the workmen themselves. I believe I am the first to devise a method whereby a burned-out block can be repaired during 65 the working of the furnace and without the necessity for interrupting the operation of the furnace or interfering with its working parts.

The essential feature of the invention is 70 that, while the furnace is working, a "center" as I term it, is inserted in position in the block, and then refractory material in a suitable plastic condition is placed or piled on or about the center so as to repair 75 the burned part, the plastic material quickly hardening under the action of the heat.

I have shown on the drawings annexed, and by way of example, a mode of carrying out the invention in connection with a Sie- 80 men's open hearth furnace.

Figure 1 is a vertical section of the open hearth furnace. Fig. 2 is a cross section taken on the line X, X, Fig. 1. Figs. 3 and 4 show means which I may use when repairing 85 a block.

On the drawings, *a* represents the furnace, *b* a working door, *c* the working bed or hearth, *d* the air port, *e*, *e*, gas ports, *f* the slag pocket, and *g* a gas regenerating cham- 90 ber.

Under my invention, when the block *i*, between the air port and a gas port (or ports) is burnt or gives way to such an extent as to render it necessary to repair the 95 same, I insert, in the gas port (or ports), while the furnace is working, what I call a "center," this center being, preferably, more or less arched or tubular in shape. The center is pushed or otherwise inserted into 100 the port (or ports). In the case of the center shown in Fig. 1, it is pushed into the gas port from the back, a hole being provided at *j* for the purpose, and which is normally closed with bricks or other stopping. 105

When the center is in place, it is easy for the workmen, by operating suitable working tools through the adjacent working door and the back opening *j*, to rebuild the block by piling on and about the center a mixture 110 made plastic by the addition of water and

consisting of broken silica brick, silver sand, and a silica clay, or other suitable refractory mixture, this being done while the furnace is working. The mixture soon hardens under the great heat while the center itself may burn away and leave the newly formed part of the block in position. In practice, I have effected a complete repair operation in about one hour. I have found, in practice, that a mixture consisting, by measure, of 50% finely broken silica brick, 20% of silver sand and 30% of a silica clay composed, by measure, of 5 parts ground silica brick and 1 part ganister, answers very well. For finishing off the rebuilt block, a mixture composed of silver sand and silica clay may be employed, these ingredients being mixed together in or about equal proportions by measure. After the mixture has been acted upon by the gas for about half an hour or so a little brown sand may be thrown on the rebuilt block so as to give a glazed surface finish.

In Fig. 1, the full lines show the block as originally built, the dotted line at  $i^1$  shows the distance to which the block may have been burnt away and the cross dotted lines at  $i^2$  show the rebuilt part of the block supported on the center  $h$ . The center may be made of metal or refractory material and may conform in section, more or less, to the shape of the port but be somewhat smaller so as to readily slip thereinto. I find, in practice, that a plate  $h^1$  of sheet iron or steel rolled to the shape shown at Figs. 3 and 4 is very suitable as it can be easily slid into place in the gas port. A fireclay pipe or a cast or wrought iron or steel tube of suitable length and shape would be equally suitable for the purpose, the object being simply to provide means sufficiently strong and fire-resisting to hold the plastic mixture in position until it hardens.

I have described the invention merely by way of illustration or example, as employed in connection with one type of regenerative open hearth furnace having a single air port and two gas ports but it is, of course, to be understood that it can be employed in connection with furnaces having two or more air ports and two or more gas ports. If two or more gas ports are burnt away then two or more centers may be used and the block re-built in the same manner as for a single port.

Having now fully described my invention, what I claim and desire to secure by Letters Patent is:—

1. The method of repairing the burnt

blocks of regenerative open hearth furnaces 60 by first inserting, in the block, a center and placing same in position where the portion of the block has been destroyed, and then applying refractory material about the center to replace the portion destroyed. 65

2. The method of repairing the burnt blocks of regenerative open hearth furnaces by providing an opening in the furnace, inserting a center through said opening and into position at the place where the block 70 has been destroyed, placing a refractory material about the center to replace the portion destroyed and thereafter closing the opening in the furnace.

3. Repairing the burnt blocks of regen- 75 erative open hearth furnaces by first inserting, in the block, a center and placing same in position where the portion of the block has been destroyed, and then applying a refractory mixture, composed of broken silica 80 brick, silver sand and clay, about the center to replace the portion destroyed.

4. Repairing the burnt blocks of regen- 85 erative open hearth furnaces by first inserting, in the block, a center and placing same in position where the portion of the block has been destroyed, then applying a mix- 90 ture of refractory material, composed of broken silica brick, silver sand and silica clay, about the center to replace the portion destroyed, and finishing off the rebuilt block with a mixture composed of silver sand and silica clay, brown sand being finally thrown on the rebuilt block for the purpose of glaz- 95 ing the same.

5. The mode of repairing the burnt blocks of regenerative open hearth furnaces by first inserting, in the block, a center, consisting of a curved plate of sheet metal, and placing same in position where the portion of the 100 block has been destroyed, and then applying a mixture of refractory material about the center to replace the portion destroyed.

6. The method of repairing the burnt blocks of regenerative open hearth furnaces 105 by first inserting, in the block, a center and placing same in position where the portion of the block has been destroyed, and then applying refractory material, in a plastic condition, about the center to replace the por- 110 tion destroyed.

In testimony whereof I affix my signature in presence of two witnesses.

THOMAS BOND ROGERSON.

Witnesses:

HUGH D. FITZPATRICK,  
WILLIAM GALL.